

1

2,758,916

## FUEL COMPOSITIONS

John E. Mahan, Bartlesville, Okla., assignor to Phillips Petroleum Company, a corporation of Delaware

No Drawing. Application July 9, 1951,  
Serial No. 235,901

19 Claims. (Cl. 44—69)

This invention relates to improved aviation fuels. More specifically it relates to an aviation fuel conforming to rigid specifications of antiknock rating, vapor pressure and distillation characteristics, and having, in addition, combustion characteristics which provide superior power output over a broad range of fuel-air ratios and particularly over the range classified as rich mixtures. It relates further to a method of operating an aviation gasoline engine requiring a fuel having an octane number of at least about 90.

High octane number aviation fuels are manufactured and blended according to specifications so strict that the selection of suitable components is limited in many cases to high purity synthetic blending stocks and naturally occurring base stocks which are segregated with such precision as to approximate the purity of the synthetic hydrocarbons. Such fuels must have high octane number ratings and this in turn means that the components must have high octane number ratings and/or excellent response to the addition of antidetonants. Further, the unsaturation of the components must be exceedingly low in order that the fuels be substantially free of gum and of susceptibility to gum formation. These qualifications together with rigid requirements for vapor pressure, end points, and distillation characteristics, sharply limit the choice of fuel components to the relatively low boiling, predominantly paraffinic hydrocarbons, say of 5 to 9 carbon atoms, and preferably to the higher octane number branched chain or isoparaffins.

In the manufacture of aviation fuels of 90 to 100 octane number or of those fuels having antiknock ratings beyond the conventional octane scale, the procedure usually includes the manufacture of synthetic isoparaffins as one blending component. For example, processes, such as selective polymerization, thermal or catalytic alkylation, or the like, may be utilized to prepare concentrates of isooctanes together with usually much smaller amounts of higher and lower homologues. Alkylation may produce such stocks as neoheptane or diisopropyl, which are highly desirable blending stocks. As a second component, base stocks comprising isohexanes, isoheptanes, isooctanes, etc., may in many instances be prepared by precise fractionation schemes from crude oil and/or natural gasolines.

A third component, which is ordinarily considered separately, is isopentane, which can be prepared in substantially pure form by fractionation of hydrocarbon mixtures containing it. This last named material is ordinarily the lowest boiling stock included in aviation fuels, and it functions as a source of volatility to adjust the vapor pressure of the blend, and to produce desirable distillation characteristics, especially in the initial portion of the distillation curve.

Since the synthetic isoparaffin blending stocks are ordinarily available in somewhat smaller volume than base stocks prepared from naturally occurring distillates, blending formulas which require minimum volumes of such synthetic stocks are preferred. Assuming that iso-

2

pentane is plentiful and used to the maximum extent possible within vapor pressure and front-end volatility limits, it then remains to select and prepare other components commonly termed base stocks of both high octane number and low vapor pressure. These characteristics are most conveniently obtained by segregation of isoparaffins, such as the isohexanes, etc., as being more valuable than a full boiling range naphtha, unless the naphtha is deficient in normal (low octane number) paraffins or has unusually high octane number as a result of its content of naphthalene hydrocarbons.

The net result of the above described blending procedure is the production of fuels of suitable distillation characteristics, vapor pressure, gum stability, and octane number rating comprising largely isoparaffins of 5 to 15 about 8 or 9 carbon atoms, substantially free of C<sub>4</sub> hydrocarbons, and preferably containing only minor amounts of C<sub>5</sub> to C<sub>9</sub> normal paraffins. The content of naphthalenes is often small, since these compounds are usually present in only small quantities or in many cases are removed more or less completely by the precise fractionation which separates the normal C<sub>5</sub>, C<sub>6</sub>, and C<sub>7</sub> paraffins from the isoparaffins in naphtha base stocks.

The complex and strenuous requirements of military aviation under war conditions have emphasized some deficiencies of aviation fuels under certain conditions. Such conditions, for example, are those which require increased or emergency power for improved and rapid take-off, particularly with heavy loads, rapid acceleration and climb during combat. The production of maximum power output under these conditions is of primary importance and the development of fuels which will meet these severe requirements under all conditions is an essential military requirement. It is also obvious that fuels which meet rigid military requirements will be of great value in the development of commercial aviation. The present invention, therefore, provides a novel fuel composition as well as mode of operating aviation engines requiring high octane fuels, particularly of 100 octane or higher. In the practice of this invention, as described herein, a gasoline essentially comprising a mixture of isoparaffin hydrocarbons having 5-9 carbon atoms per molecule, containing TEL, usually at least about 3 ml. per gallon, together with a minor proportion of an additive material, preferably 1-10 per cent, and having a Reid vapor pressure not greater than about seven pounds, and a maximum 90 per cent ASTM distillation procedure evaporated temperature of about 275° F., is supplied to an aviation engine during an operating period, and particularly when rich mixture performance is required.

50 The term "rich mixture performance" as now used by the art, and as referred to herein, describes the power output of aviation engines under rich mixture conditions, such, for example, as would be obtained by substantially increasing the fuel concentration in an air-fuel mixture 55 at the intake of an aviation engine. This performance is usually defined in terms relating to a standard 100 octane number reference fuel, the relative improvement being stated in ml. of tetraethyl lead.

Use of multiple engines in aircraft has often necessitated the overloading of a portion of the engines by reason of the fact that another portion of the engines may cease to operate during flight. At such times, it has been found to be very desirable to have a fuel which will give an increased power output over that normally utilized under cruising conditions. Additional power output has also been found to be necessary for take-off and high rate of climb of aircraft when operating at fuel-air ratios much higher than the lean mixture ratios ordinarily employed for cruising operation. By reason of the necessity for such increased power output, a new consideration for blending formulas has been introduced

for the purpose of increasing the potential power output of finished fuels.

Isoparaffinic fuel compositions generally are very satisfactory from the standpoint of most specifications when it is not necessary to utilize additional power over that normally required under lean mixture ratios used under cruising conditions. Use of these isoparaffinic fuels permits the production of larger volumes of finished fuel per volume of synthetic blending stocks than are possible with other blending formulas. It is thus ordinarily most advantageous to retain the isoparaffin blending formulas insofar as possible. This procedure requires that such special performance characteristics as lean and rich mixture ratings be obtained through the inclusion of minor proportions of substantially pure chemical additives. These additive compounds must be carefully selected so that the desired improvements are obtained with such small quantities that other fuel characteristics are not impaired and blend specifications are not infringed.

An object of this invention is to provide an improved fuel composition for use in aircraft engines whereby the effective operation and power output of the engines are improved. Another object of the invention is to provide an improvement in the blending formula for preparing predominantly isoparaffinic aviation fuels whereby the potential power output thereof is greatly increased. Another object of this invention is to provide an isoparaffinic aviation fuel of at least 90-leaded aviation octane number rating containing a relatively minor proportion of an added compound providing greatly improved power output characteristics without undesirably effecting the other characteristics of the fuel. Another object is to provide an isoparaffinic aviation fuel of about 100 aviation octane number rating or better containing a relatively minor proportion of an added compound providing greatly improved rich mixture characteristics without undesirably affecting the other characteristics of the fuel. Another object is to provide a fuel composition comprising an aviation base stock containing a relatively minor proportion of a selected monoalkenylamine. Another object is to provide an improved method for operating aviation engines under conditions requiring increased power output by the addition to the isoparaffinic aviation fuel utilized therein a minor proportion of a selected monoalkenylamine. Other objects will be apparent to one skilled in the art from the accompanying discussion and disclosure.

I have found that aviation fuels of the type described and comprising essentially isoparaffinic hydrocarbons have greatly improved power output ratings particularly over the rich mixture range of fuel-air ratios, when they contain minor proportions of monoalkenylamines characterized by the structural formula



wherein X is an alkenyl radical of branched or straight chain configuration containing from 3 to 8 carbon atoms, and R and R' can each be hydrogen,  $\text{CH}_3$ , or  $\text{C}_2\text{H}_5$ , and the sum of the carbon atoms in the R and R' does not exceed 2; the alkenyl radical is preferably monoolefinic, i. e., containing one olefinic carbon-to-carbon bond, although in some instances it may contain 2 or even 3 olefinic bonds. The mono substituted amines such as butenylamine, pentenylamine, hexenylamine, and the like are preferred additive compounds of my invention. However, di- or tri-substituted amines such as N-methylbutenylamine, N,N-dimethylpentenylamine and the like are adaptable as fuel additives, and are within the scope of my invention.

The unsaturated amines described above are employed as substantially pure compounds or mixtures of these pure compounds, since their efficiency is highly specific

and superior to certain other nitrogen compounds which might be present in crude unsaturated amine fractions. A further purpose served by the use of substantially pure compounds or mixtures thereof is the elimination of associated impurities which have deteriorative effects on the fuel and/or aircraft fuel systems in which it is used.

In addition to the unsaturated monoalkenylamines applicable in the process of my invention, already named, are included N-ethyloctenylamine, N,N-dimethylheptenylamine, N-ethylpentenylamine, N-methylpropenylamine, N,N-dimethylbutenylamine, allylamine, heptenylamine, iso-octenylamine, N-methylisopentenylamine, N,N-dimethylisobutylamine, and the like. These compounds are exemplary of those unsaturated amines which in accordance with my invention, when added to an aviation fuel of the type described, improve the rich mixture performance of the fuel, as determined by the supercharged engine test (AN-VV-F-748a).

While specific embodiments of the present invention may be invoked in a great variety of blending operations involving isoparaffinic blending and base stocks, one satisfactory procedure is outlined in the following operations. A fuel is prepared according to a blending formula from isooctane, isopentane and a naphtha comprising  $\text{C}_6$  and  $\text{C}_7$  isoparaffins in proportions which produce 100 octane number with 4 ml. of tetraethyl lead per gallon. This formula is altered according to the present invention to include at least one of the unsaturated amines described above by use of a predetermined volume per cent of an unsaturated amine-pentane mixture having a vapor pressure substantially equal to that of the finished fuel (usually about seven pounds Reid vapor pressure). The volume of a mixture used replaces a corresponding volume of isoparaffin base stock and synthetic blending stock with the blending proportions of the latter ordinarily being readjusted to produce the same aviation octane number rating as before.

The unsaturated amine additives may be added alone to fuel blends, but it is often more convenient to employ the isopentanized mixture. The advantages lie in the maximum utilization of the isoparaffin ingredients, particularly isopentane, and less difficulty in blending to meet vapor pressure specifications, and in improving the rich rating of the fuel.

The unsaturated amines described above may be prepared in any desired manner. One such specific preparation is described in the copending application of J. E. Mahan and K. F. Bursack, Serial No. 135,290, filed December 27, 1949, now abandoned. In accordance with the process disclosed in that copending application a conjugated hydrocarbon diene containing at least 4 carbon atoms in the molecule is reacted with ammonia or an organic amine in liquid phase in the presence of sodium hydride or sodamide as a catalyst to form the monoalkenylamine, together with di- and trialkenyl products. Accordingly in the preparation of monobutenylamine, 1,3-butadiene is reacted with ammonia in the presence of the catalyst. Operating temperatures are from 50- to 500° F., temperatures approximating 100° F. being often desirable. It is understood, of course, that monobutenylamines as well as other unsaturated amines applied to the process of my invention can be prepared in any suitable manner although for reasons described above I prefer generally that the additive to be employed is applied in a high state of purity.

The proportions of the above described unsaturated amine additives to be added to the fuel will obviously be dependent on the other fuel components and on the particular lean mixture and rich mixture octane ratings which are desired in the final blend. In most cases the quantity of the unsaturated amine additive employed will be in the range of from 1 to 10 volume per cent of the finished fuel.

The amine additives in accordance with my invention

are applied to both clear and leaded fuels, although my preferred fuel compositions contain tetraethyl lead in proportions generally from 3.0 to 4.6 ml. per gallon; however, proportions of tetraethyl lead outside the preferred range can be employed as desired, as for example proportions as low as about 1 ml./gallon and as high as 7 ml./gallon. The unsaturated amine additives described above exhibit water solubility and generally when applied in the practice of my invention the maximum concentration of additive that can be used will be equal to the amount that will provide a finished fuel which passes the maximum water tolerance concentration as determined for example by the test AN-F-48b. This amount on a volume basis is at least 1 per cent, and preferably at least 1.5 per cent and generally does not exceed 10 per cent, although in cases where a larger amount can be used and the fuel passes the said water tolerance test, the use of a larger amount is within the scope of my invention.

In another embodiment of my invention I am able to take particular advantage of the water solubility of the above described unsaturated amine additives, inasmuch as appreciable quantities of water can thus be incorporated with the finished fuel to aid in knock suppression and to aid in alleviating formation of piston and cylinder deposits.

In another embodiment of my invention the solubility of the unsaturated amine additive in water can be utilized by injecting the additive into the combustion system in the form of a water solution when needed, in a manner generally analogous to the use of water injection at high powers. These latter embodiments of my invention, as applied to the water solubility characteristics described, are particularly applicable when applying monobutenylamines as the desired unsaturated amine.

Test method AN-VV-F-746 as referred to herein is the method identified as Army-Navy Aeronautical Specification Fuel: Aircraft Engine General Specification (Method for Knock-Test AN-VV-F-746), dated October 5, 1940. This method is utilized for determining ordinary aviation octane number ratings of aviation fuels. Test method AN-VV-F-748a, as referred to herein is identified as Army-Navy Aeronautical Specification Fuel; Aircraft Engine, General Specification (Method for Supercharged Knock-Test) AN-VV-F-748a dated June 17, 1942. The test method described therein is used for determining lean and rich mixture ratings of 100 octane number aviation fuels. In this latter specification (AN-VV-F-748a) a lean mixture is shown to be about 0.06 pound of fuel per pound of air and a rich mixture at least about 0.09 pound of fuel per pound of air.

More recently, however, it has been shown that while this latter method (AN-VV-F-748a) can be used to give an excellent measure of the performance of fuels in rich mixtures, lean mixture ratings obtained in this supercharged engine test are erratic and unreliable. At

the present time the aviation octane ratings obtained in the ordinary aircraft engine tests (AN-VV-F-746 and ASTM Aviation method D-614-48T) which are carried out under lean mixture conditions, are considered a more reliable measure of lean mixture performance and the lean mixture ratings obtained in the supercharged test have fallen into disuse.

It has been found that it is generally not possible to add directly the rich mixture ratings of the components of an 10 aviation fuel blend in their volumetric proportions and arrive at a correct value for the rating of the blend, or conversely, from the rating of the blend to determine the value of the additive. This is particularly true where the components differ widely in their rating, and results in 15 part from the conventions used in expressing rich ratings. While rich ratings superior to the performance of isoocetane are given in terms of the value of tetraethyl lead that must be added to reference fuel S (essentially pure isoocetane) to reproduce the same engine performance, rich ratings inferior to isoocetane are expressed in terms of the volume per cent of fuel S in a blend with reference fuel M (low octane straight run gasoline) to reproduce the engine performance. To reconcile these two methods of expression and the non-linearity of the concentration-performance relationship, the procedure has been 20 adopted of assigning a number known as the "rich mixture blending index" number to measurable performance levels. These numbers are so assigned and tabulated that they may be used directly with the volumetric percentage of the constituents to give the performance rating of the blend. Thus, a fuel of very poor performance, which is equivalent to a blend of 83.0 per cent fuel S in fuel M has a blending index number of 4. Pure isoocetane has a blending index number of 100, while a 25 superior fuel whose performance is equal to that of isoocetane with 6.0 cc. of lead added has a blending index number of 162.

As illustrations of the improved performance characteristics obtained by the addition of monoalkenylamines 30 in isoparaffinic aviation fuels, the following example is cited.

#### Example 1

Three portions of a 91/98 aviation base stock were 45 blended with monobutenylamine. A portion of the unblended 91/98 stock and each of the three resulting blends were subjected to octane number and rich rating tests. Similarly a portion of a 100/130 grade aviation base stock was blended with monobutenylamine and another portion of the same base stock was blended with monoallylamine, and, a portion of the unblended 100/130 base stock and each of the resulting blends thereof, were subjected to octane number and rich rating tests. Details and results of these tests are summarized in the tabulation below:

| Formula | Composition                            |                                          |                  |               | ASTM Aviation Octane Number (4.0 ml. TEL) | Aviation Blending Octane Number (4.0 ml. TEL) | ASTM Supercharge <sup>a</sup> Rich Rating (4.0 ml. TEL) | ASTM Supercharge Rich Mixture Blending Index Number (4.0 ml. TEL) |
|---------|----------------------------------------|------------------------------------------|------------------|---------------|-------------------------------------------|-----------------------------------------------|---------------------------------------------------------|-------------------------------------------------------------------|
|         | Grade 91/98 Aviation Base <sup>b</sup> | Grade 100/130 Aviation Base <sup>b</sup> | Monobutenylamine | Monallylamine |                                           |                                               |                                                         |                                                                   |
| 1       | 100.0                                  |                                          |                  |               | 92.2                                      |                                               | 197.2                                                   |                                                                   |
| 2       | 95.0                                   |                                          | 5.0              |               |                                           |                                               | • 0.09                                                  | 442.8                                                             |
| 3       | 95.0                                   |                                          | 5.0              |               | 91.5                                      | 78.2                                          | 199.5                                                   | 340.8                                                             |
| 4       | 95.0                                   |                                          | 5.0              |               | 92.0                                      | 88.2                                          | 199.4                                                   | 332.8                                                             |
| 5       |                                        | 100.0                                    |                  |               | 100.0                                     |                                               | • 1.32                                                  |                                                                   |
| 6       |                                        | 98.0                                     | 2.0              |               | 98.1                                      | 5.0                                           | • 1.38                                                  | 161.0                                                             |
| 7       |                                        | 95.0                                     |                  | 5.0           | 100.0                                     | 100.0                                         | • 1.39                                                  | 145.0                                                             |

<sup>a</sup> 14.4 percent iC<sub>8</sub> base stock + 41.3 percent iC<sub>7</sub> + 31.3 percent iC<sub>6</sub> + 13.0 percent iC<sub>5</sub>.  
<sup>b</sup> 50 percent HF alkylate + 9.7 percent mixed cyclers + 11.0 percent iC<sub>7</sub> + 12.7 percent iC<sub>8</sub> base stock + 16.6 percent iC<sub>5</sub>.

<sup>a</sup> Determined in accordance with Test Method D-614-48T, described hereinabove.

<sup>b</sup> Determined in accordance with Test Method AN-VV-F-748a, described hereinabove.

<sup>a</sup> ml. of TEL that must be added to isoocetane (2,2,3-trimethylpentane).

<sup>b</sup> Volume percent isoocetane (2,2,3-trimethylpentane) in n-heptane.

The data of the preceding example demonstrate the substantially improved rich mixture characteristics of the fuel, resulting from the addition thereto of monobutenylamine and monoallylamine. These improved ratings are particularly manifest by the tabulated rich mixture index numbers.

*Example II*

A portion of a 91/98 aviation base stock was blended with diallylamine. The resulting blend, and a separate portion of the 91/98 base stock were subjected to rich rating tests. Details and results of these tests are summarized in the tabulation below:

| Composition  |                                        | ASTM Supercharge Rich Rating (4.0 ml. TEL) | ASTM Supercharge Rich blending Index No. (4.0 ml. TEL) |
|--------------|----------------------------------------|--------------------------------------------|--------------------------------------------------------|
| Diallylamine | Grade 91/98 aviation base <sup>1</sup> |                                            |                                                        |
| 5            | 100<br>95                              | 97.2<br>96.6                               | 8.8                                                    |
|              |                                        |                                            |                                                        |

<sup>1</sup> 14.4 percent, IC<sub>8</sub> base stock + 41.3 percent IC<sub>7</sub> + 31.3 percent IC<sub>6</sub> + 13.0 percent IC<sub>5</sub>.

The above tabulated data illustrate that diallylamines cannot be considered as equivalents of monoalkenylamines in effecting improvement in rich-mixture characteristics of aviation fuels. This is particularly demonstrated by the low blending index number of 8.8 as determined for diallylamine as compared to the blending index number of 145 as determined for monoallylamine, set forth in Example I above.

As will be evident to those skilled in the art, various modifications can be made or followed, in the light of the foregoing disclosure and discussion, without departing from the spirit or scope of the disclosure or from the scope of the claims.

I claim:

1. A gasoline containing from 1 to 10 volume per cent of at least one unsaturated amine characterized by the structural formula



wherein X is an alkenyl radical containing from 3 to 8 carbon atoms, R and R' are each radicals selected from the group consisting of hydrogen, CH<sub>3</sub> and C<sub>2</sub>H<sub>5</sub>, and wherein the number of carbon atoms in the total R and R' radicals does not exceed 2.

2. A gasoline according to claim 1 wherein said amine is monopentenylamine.

3. A gasoline according to claim 1 wherein said amine is monohexenylamine.

4. A gasoline according to claim 1 wherein said amine is N-methylbutenylamine.

5. An improved gasoline containing from 1 to 10 volume per cent of monobutenylamine.

6. An improved gasoline containing from 1 to 10 volume per cent of monoallylamine.

7. An improved gasoline consisting essentially of an aviation base stock, including a substantial proportion of isoparaffinic hydrocarbons having from 5 to 9 carbon atoms in the molecule, a small proportion of tetraethyl lead, and from 1 to 10 per cent of its volume of at least one unsaturated amine characterized by the structural formula



wherein X is an alkenyl radical containing from 3 to 8 carbon atoms, and R and R' are each radicals selected from the group consisting of hydrogen, CH<sub>3</sub> and C<sub>2</sub>H<sub>5</sub>, and wherein the number of carbon atoms in the total R and R' radicals does not exceed 2.

8. An improved gasoline consisting essentially of a small proportion of tetraethyl lead, an aviation base stock, including a substantial proportion of isoparaffinic hydrocarbons having from 5 to 9 carbon atoms in the molecule, and from 1 to 10 volume per cent of monobutenylamine, and having a maximum Reid vapor pressure of seven pounds and a maximum 90 per cent ASTM evaporated temperature of 275° F.

9. An improved gasoline consisting essentially of a small proportion of tetraethyl lead, an aviation base stock, including a substantial proportion of isoparaffinic hydrocarbons having from 5 to 9 carbon atoms in the molecule, and from 1 to 10 volume per cent of monoallylamine, and having a maximum Reid vapor pressure of seven pounds, and a maximum 90 per cent ASTM evaporated temperature of 275° F.

10. An improved gasoline consisting essentially of a grade 100/130 aviation base stock containing a small proportion of tetraethyl lead and from 1 to 10 volume per cent monobutenylamine.

11. An improved gasoline consisting essentially of a grade 100/130 aviation base stock containing a small proportion of tetraethyl lead and from 1 to 10 volume per cent monoallylamine.

12. An improved gasoline consisting essentially of a grade 91/98 aviation base stock containing a small proportion of tetraethyl lead and from 1 to 10 volume per cent monobutenylamine.

13. An improved gasoline consisting essentially of a grade 91/98 aviation base stock containing a small proportion of tetraethyl lead and from 1 to 10 volume per cent monoallylamine.

14. A gasoline containing a minor proportion, in an amount sufficient to increase the rich mixture blending index number of said gasoline, of at least one unsaturated amine characterized by the structural formula



wherein X is an alkenyl radical containing from 3 to 8 carbon atoms, R and R' are each radicals selected from the group consisting of hydrogen, CH<sub>3</sub> and C<sub>2</sub>H<sub>5</sub>, and wherein the number of carbon atoms in the total R and R' radicals does not exceed 2.

15. A gasoline according to claim 14 wherein said amine is monobutenylamine.

16. A gasoline according to claim 14 wherein said amine is monoallylamine.

17. A gasoline according to claim 14 wherein said amine is monopentenylamine.

18. A gasoline according to claim 14 wherein said amine is monohexenylamine.

19. A gasoline according to claim 14 wherein said amine is N-methylbutenylamine.

References Cited in the file of this patent

UNITED STATES PATENTS

|           |                      |                |
|-----------|----------------------|----------------|
| 1,724,640 | Calcott et al. ----- | Aug. 13, 1929  |
| 1,992,014 | Rogers et al. -----  | Feb. 19, 1935  |
| 2,021,088 | Pevere -----         | Nov. 12, 1935  |
| 2,324,118 | Sweeney -----        | July 13, 1943  |
| 2,618,612 | Howell -----         | Nov. 18, 1952  |
| 2,653,862 | Trimble et al. ----- | Sept. 29, 1953 |